



US008119316B2

(12) **United States Patent**  
Lin et al.

(10) **Patent No.:** **US 8,119,316 B2**  
(45) **Date of Patent:** **Feb. 21, 2012**

(54) **THIURAM TETRASULFIDE CONTAINING PHOTOGENERATING LAYER**

(75) Inventors: **Liang-Bih Lin**, Rochester, NY (US); **Daniel V Levy**, Philadelphia, PA (US); **Jin Wu**, Webster, NY (US); **Markus R Silvestri**, Fairport, NY (US)

(73) Assignee: **Xerox Corporation**, Norwalk, CT (US)

(\*) Notice: Subject to any disclaimer, the term of this patent is extended or adjusted under 35 U.S.C. 154(b) by 864 days.

(21) Appl. No.: **12/059,448**

(22) Filed: **Mar. 31, 2008**

(65) **Prior Publication Data**

US 2009/0246658 A1 Oct. 1, 2009

(51) **Int. Cl.**

**G03G 5/047** (2006.01)

(52) **U.S. Cl.** ..... **430/58.8**; 430/58.65; 430/58.75; 430/59.1; 430/59.4; 430/59.5; 430/64

(58) **Field of Classification Search** ..... 430/58.65, 430/58.75, 58.8, 59.1, 59.4, 59.5, 64

See application file for complete search history.

(56) **References Cited**

U.S. PATENT DOCUMENTS

|                |         |                              |
|----------------|---------|------------------------------|
| 4,265,990 A    | 5/1981  | Stolka et al.                |
| 4,298,697 A    | 11/1981 | Baczek et al.                |
| 4,338,390 A    | 7/1982  | Lu                           |
| 4,464,450 A    | 8/1984  | Teuscher                     |
| 4,560,635 A    | 12/1985 | Hoffend et al.               |
| 4,587,189 A    | 5/1986  | Hor et al.                   |
| 4,921,773 A    | 5/1990  | Melnik et al.                |
| 5,482,811 A    | 1/1996  | Keoshkerian et al.           |
| 5,521,306 A    | 5/1996  | Burt et al.                  |
| 6,913,863 B2   | 7/2005  | Wu et al.                    |
| 7,018,756 B2 * | 3/2006  | Pai et al. .... 430/58.65    |
| 7,125,633 B2 * | 10/2006 | Mishra et al. .... 430/58.3  |
| 7,344,809 B2 * | 3/2008  | Horgan et al. .... 430/58.75 |
| 7,410,738 B2 * | 8/2008  | Yanus et al. .... 430/58.5   |

2004/0126685 A1 \* 7/2004 Horgan et al. .... 430/58.3  
2007/0026330 A1 \* 2/2007 Wu et al. .... 430/58.05  
2007/0298342 A1 \* 12/2007 Wu et al. .... 430/58.75

FOREIGN PATENT DOCUMENTS

JP 09319121 A \* 12/1997

OTHER PUBLICATIONS

Liang-Bih Lin et al., U.S. Appl. No. 12/059,478 on Benzothiazole Containing Photogenerating Layer, filed concurrently herewith.

Jin Wu et al., U.S. Appl. No. 12/059,448 on Thiuram Tetrasulfide Containing Photogenerating Layer, filed concurrently herewith.

Jin Wu et al., U.S. Appl. No. 12/059,525 on Additive Containing Photoconductors, filed concurrently herewith.

Jin Wu et al., U.S. Appl. No. 12/059,536 on Carbazole Hole Blocking Layer Photoconductors, filed concurrently herewith.

Jin Wu et al., U.S. Appl. No. 12/059,573 on Oxadiazole Containing Photoconductors, filed concurrently herewith.

Jin Wu et al., U.S. Appl. No. 12/059,587 on Titanocene Containing Photoconductors, filed concurrently herewith.

Jin Wu et al., U.S. Appl. No. 12/059,663 on Thiadiazole Containing Photoconductors, filed concurrently herewith.

Jin Wu et al., U.S. Appl. No. 12/059,669 on Overcoat Containing Titanocene Photoconductors, filed concurrently herewith.

Daniel Levy et al., U.S. Appl. No. 12/059,546 on Urea Resin containing Photogenerating Layer Photoconductors, filed concurrently herewith.

Jin Wu et al., U.S. Appl. No. 12/059,689 on Metal Oxide Overcoated Photoconductors, filed concurrently herewith.

Jin Wu et al., U.S. Appl. No. 11/869,252 on Additive Containing charge Transport Layer Photoconductors, filed Oct. 9, 2007.

Liang-Bih Lin et al., U.S. Appl. No. 11/800,129 on Photoconductors, filed May 4, 2007.

Liang-Bih Lin et al., U.S. Appl. No. 11/800,108 on Photoconductors, filed May 4, 2007.

\* cited by examiner

*Primary Examiner* — Peter Vajda

(74) *Attorney, Agent, or Firm* — Oliff & Berridge, PLC

(57) **ABSTRACT**

A photoconductor comprising a supporting substrate, a photogenerating layer, and at least one charge transport layer comprised of at least one charge transport component, and wherein the photogenerating layer contains a thiuram sulfide additive.

**12 Claims, No Drawings**

## THIURAM TETRASULFIDE CONTAINING PHOTOGENERATING LAYER

### CROSS REFERENCE TO RELATED APPLICATIONS

U.S. application Ser. No. 12/059,478, U.S. Publication No. 20090246659, filed Mar. 31, 2008 on Benzothiazole Containing Photogenerating Layer, the disclosure of which is totally incorporated herein by reference.

U.S. application Ser. No. 12/059,555, U.S. Publication No. 20090246662, filed Mar. 31, 2008 on Hydroxyquinoline Containing Photoconductors, the disclosure of which is totally incorporated herein by reference.

U.S. application Ser. No. 12/059,525, U.S. Publication No. 20090246660, filed Mar. 31, 2008 on Additive Containing Photoconductors, the disclosure of which is totally incorporated herein by reference.

U.S. application Ser. No. 12/059,536, now U.S. Pat. No. 7,794,906, filed Mar. 31, 2008 on Carbazole Hole Blocking Layer Photoconductors, the disclosure of which is totally incorporated herein by reference.

U.S. application Ser. No. 12/059,573, U.S. Publication No. 20090246664, filed Mar. 31, 2008 on Oxadiazole Containing Photoconductors, the disclosure of which is totally incorporated herein by reference.

U.S. application Ser. No. 12/059,587, now U.S. Pat. No. 7,811,732, filed Mar. 31, 2008 on Titanocene Containing Photoconductors, the disclosure of which is totally incorporated herein by reference.

U.S. application Ser. No. 12/059,663, U.S. Publication No. 20090246666, filed Mar. 31, 2008 on Thiadiazole Containing Photoconductors, the disclosure of which is totally incorporated herein by reference.

U.S. application Ser. No. 12/059,669, U.S. Publication No. 20090246657, filed Mar. 31, 2008 on Overcoat Containing Titanocene Photoconductors, the disclosure of which is totally incorporated herein by reference.

U.S. application Ser. No. 12/059,546, U.S. Publication No. 20090246661, filed Mar. 31, 2008 on Urea Resin Containing Photogenerating Layer Photoconductors, the disclosure of which is totally incorporated herein by reference.

U.S. application Ser. No. 12/059,689, now U.S. Pat. No. 7,799,495, filed Mar. 31, 2008 on Metal Oxide Overcoated Photoconductors, the disclosure of which is totally incorporated herein by reference.

U.S. application Ser. No. 11/869,252, U.S. Publication No. 20090092911 by Jin Wu et al. on Additive Containing Charge Transport Layer Photoconductors, the disclosure of which is totally incorporated herein by reference, there is disclosed a photoconductor comprising a supporting substrate, a photogenerating layer, and at least one charge transport layer comprised of at least one charge transport component, and an ammonium salt additive or dopant.

U.S. application Ser. No. 11/800,129, U.S. Publication No. 20080274419 filed May 4, 2007 by Liang-Bih Lin et al. on Photoconductors, the disclosure of which is totally incorporated herein by reference, there is illustrated a photoconductor comprising a supporting substrate, a photogenerating layer, and at least one charge transport layer comprised of at least one charge transport component, and wherein the photogenerating layer contains a bis(pyridyl)alkylene.

U.S. application Ser. No. 11/800,108, now U.S. Pat. No. 7,662,526, filed May 4, 2007 by Liang-Bih Lin et al. on Photoconductors, the disclosure of which is totally incorporated herein by reference, there is disclosed a photoconductor comprising a supporting substrate, a photogenerating layer,

and at least one charge transport layer comprised of at least one charge transport component, and wherein the charge transport layer contains a benzimidazole.

### BACKGROUND

This disclosure is generally directed to imaging members, photoreceptors, photoconductors, and the like. More specifically, the present disclosure is directed to multilayered drum, or flexible, belt imaging members, or devices comprised of a supporting medium like a substrate, a photogenerating layer, and a charge transport layer, including a plurality of charge transport layers, such as a first charge transport layer and a second charge transport layer, and wherein the photogenerating layer contains a thiuram sulfide, especially tetrasulfide additive or dopant, and a photoconductor comprised of a supporting medium like a substrate, a photogenerating layer, and a charge transport layer, including a plurality of charge transport layers, such as a first charge transport layer and a second charge transport layer, and wherein the photogenerating layer includes an additive of a thiuram tetrasulfide, such as dipentamethylenethiuram tetrasulfide (DPTT) especially in powder form, and which additive is substantially soluble in a number of solvents selected for the preparation of the photogenerating layer, such as a solvent including tetrahydrofuran.

The additives or dopants, which can be incorporated into the photogenerating layer, and which dopants function, for example, to passivate the photogenerating pigment surface by, for example, blocking or substantially blocking intrinsic free carriers, and preventing or minimizing external free carriers from being attracted to the pigment surface, permit photoconductors with excellent ghosting characteristics, that is where there is minimal ghosting as compared to a similar photoconductor without the additive. Also, it is believed that with the additive there may be achievable photoconductors with minimal CDS (charge deficient spots), the control of the PIDC, for example tuning, and reducing the PIDC especially in those situations where the photosensitivity of the photoconductor can be adjusted on line and automatically to a desired preselected value or amount, and which photosensitivity can be increased or decreased; and acceptable LCM characteristics, such as for example improved lateral charge migration (LCM) resistance.

Also included within the scope of the present disclosure are methods of imaging and printing with the photoconductor devices illustrated herein. These methods generally involve the formation of an electrostatic latent image on the imaging member, followed by developing the image with a toner composition comprised, for example, of thermoplastic resin, colorant, such as pigment, charge additive, and surface additives, reference U.S. Pat. Nos. 4,560,635; 4,298,697 and 4,338,390, the disclosures of which are totally incorporated herein by reference, subsequently transferring the image to a suitable substrate, and permanently affixing the image thereto. In those environments wherein the device is to be used in a printing mode, the imaging method involves the same operation with the exception that exposure can be accomplished with a laser device or image bar. More specifically, the imaging members and flexible belts disclosed herein can be selected for the Xerox Corporation iGEN3® machines that generate with some versions over 100 copies per minute. Processes of imaging, especially xerographic imaging and printing, including digital and/or color printing, are thus encompassed by the present disclosure.

The photoconductors disclosed herein are in embodiments sensitive in the wavelength region of, for example, from about

400 to about 900 nanometers, and in particular from about 650 to about 850 nanometers, thus diode lasers can be selected as the light source. Moreover, the imaging members disclosed herein are in embodiments useful in high resolution color xerographic applications, particularly high-speed color copying and printing processes.

## REFERENCES

There is illustrated in U.S. Pat. No. 6,913,863, the disclosure of which is totally incorporated herein by reference, a photoconductive imaging member comprised of a hole blocking layer, a photogenerating layer, and a charge transport layer, and wherein the hole blocking layer is comprised of a metal oxide; and a mixture of a phenolic compound and a phenolic resin wherein the phenolic compound contains at least two phenolic groups.

Layered photoconductors have been described in numerous U.S. patents, such as U.S. Pat. No. 4,265,990, the disclosure of which is totally incorporated herein by reference, wherein there is illustrated an imaging member comprised of a photogenerating layer, and an aryl amine hole transport layer.

In U.S. Pat. No. 4,587,189, the disclosure of which is totally incorporated herein by reference, there is illustrated a layered imaging member with, for example, a perylene, pigment photogenerating component and an aryl amine component, such as N,N'-diphenyl-N,N'-bis(3-methylphenyl)-1,1'-biphenyl-4,4'-diamine dispersed in a polycarbonate binder as a hole transport layer.

Illustrated in U.S. Pat. No. 5,521,306, the disclosure of which is totally incorporated herein by reference, is a process for the preparation of Type V hydroxygallium phthalocyanine comprising the in situ formation of an alkoxy-bridged gallium phthalocyanine dimer, hydrolyzing the dimer to hydroxygallium phthalocyanine, and subsequently converting the hydroxygallium phthalocyanine product to Type V hydroxygallium phthalocyanine.

Illustrated in U.S. Pat. No. 5,482,811, the disclosure of which is totally incorporated herein by reference, is a process for the preparation of hydroxygallium phthalocyanine photogenerating pigments which comprises as a first step hydrolyzing a gallium phthalocyanine precursor pigment by dissolving the hydroxygallium phthalocyanine in a strong acid and then reprecipitating the resulting dissolved pigment in basic aqueous media.

Also, in U.S. Pat. No. 5,473,064, the disclosure of which is totally incorporated herein by reference, there is illustrated a process for the preparation of photogenerating pigments of hydroxygallium phthalocyanine Type V essentially free of chlorine, whereby a pigment precursor Type I chlorogallium phthalocyanine is prepared by reaction of gallium chloride in a solvent, such as N-methylpyrrolidone, present in an amount of from about 10 parts to about 100 parts, and preferably about 19 parts with 1,3-diiminoisoindolene (DI<sup>3</sup>) in an amount of from about 1 part to about 10 parts, and preferably about 4 parts of DI<sup>3</sup>, for each part of gallium chloride that is reacted; hydrolyzing said pigment precursor chlorogallium phthalocyanine Type I by standard methods, for example acid pasting, whereby the pigment precursor is dissolved in concentrated sulfuric acid and then reprecipitated in a solvent, such as water, or a dilute ammonia solution, for example from about 10 to about 15 percent; and subsequently treating the resulting hydrolyzed pigment hydroxygallium phthalocyanine Type I with a solvent, such as N,N-dimethylformamide, present in an amount of from about 1 volume part to about 50 volume parts, and more specifically, about 15 volume parts

for each weight part of pigment hydroxygallium phthalocyanine that is used by, for example, ball milling the Type I hydroxygallium phthalocyanine pigment in the presence of spherical glass beads, approximately 1 millimeter to 5 millimeters in diameter, at room temperature, about 25° C., for a period of from about 12 hours to about 1 week, and more specifically, about 24 hours.

The appropriate components, such as the supporting substrates, the photogenerating layer components, the charge transport layer components, the overcoating layer components, and the like of the above recited patents, may be selected for the photoconductors of the present disclosure in embodiments thereof.

## SUMMARY

Disclosed are imaging members and photoconductors that contain a dopant in the photogenerating layer, and where there are permitted preselected electrical characteristics, and more specifically, acceptable PIDC values; excellent minimal ghosting characteristics on, for example, xerographic prints or copies; excellent lateral charge migration (LCM) resistance, and excellent cyclic stability properties.

Additionally disclosed are flexible belt imaging members containing optional hole blocking layers comprised of, for example, amino silanes (throughout in this disclosure plural also includes nonplural, thus there can be selected a single amino silane), metal oxides, phenolic resins, and optional phenolic compounds, and which phenolic compounds contain at least two, and more specifically, two to ten phenol groups or phenolic resins with, for example, a weight average molecular weight ranging from about 500 to about 3,000, permitting, for example, a hole blocking layer with excellent efficient electron transport which usually results in a desirable photoconductor low residual potential  $V_{low}$ .

The photoconductors illustrated herein, in embodiments, have excellent wear resistance, extended lifetimes, elimination or minimization of imaging member scratches on the surface layer or layers of the member, and which scratches can result in undesirable print failures where, for example, the scratches are visible on the final prints generated. Additionally, in embodiments the photoconductors disclosed herein possess excellent, and in a number of instances low  $V_r$  (residual potential), and allow the substantial prevention of  $V_r$  cycle up when appropriate; low acceptable image ghosting characteristics; low background and/or minimal charge deficient spots (CDS); and desirable toner cleanability. At least one in embodiments refers, for example, to one, to from 1 to about 10, to from 2 to about 7; to from 2 to about 4, to two, and the like.

## EMBODIMENTS

Aspects of the present disclosure relate to a photoconductor comprising a supporting substrate, a photogenerating layer, and at least one charge transport layer comprised of at least one charge transport component, and where the photogenerating layer contains the additive or dopant as illustrated herein; a flexible photoconductive imaging member comprised in sequence of a supporting substrate, an additive containing photogenerating layer thereover, a charge transport layer, and a protective top overcoating layer; a photoconductor which includes a hole blocking layer and an adhesive layer where the adhesive layer is situated between the hole blocking layer and the photogenerating layer, and the hole blocking layer is situated between the substrate and the adhesive layer; and a photoconductor wherein the additive or dopant can be

selected in various effective amounts, such as for example, in parts per million, like from about 1 to about 1,000, and from about 10 to about 500 parts per million of the additive.

Examples of the additive or dopant present, for example, in various amounts, such as from about 0.1 to about 25, from about 1 to about 15, from about 2 to about 7 weight percent, include, for example, a number of known suitable components, such as alkylalkylene thiuram sulfides, especially disulfides like a thiuram tetrasulfide, a class of known accelerators materials used in the rubber industry.

Examples of thiuram sulfide additives include dipentamethylenethiuram tetrasulfide (DPTT), which can be obtained from Flexsys Corporation and U.S. Rubber Corporation; a thiuram sulfide represented by at least one of the following



wherein each R is independently selected from the group consisting of at least one of hydrogen, alkyl with, for example, from about 1 to about 40 carbon atoms; alkoxy with, for example, from about 1 to about 40 carbon atoms; aryl with, for example, from about 6 to about 30 carbon atoms, such as phenyl, substituted phenyl; pyridyl, substituted pyridyl; higher aromatics, such as naphthalene and anthracene; alkylphenyl with up to about 40 carbon atoms; alkoxyphenyl with, for example, from about 6 to about 40 carbon atoms; aryl with, for example, from about 6 to about 30 carbon atoms; substituted aryl with, for example, from about 7 to about 30 carbons, and halogen; and x represents the number of sulfur atoms, which number can be, for example, from 1 to about 8.

Further examples of the additive include thiuram sulfide derivatives represented by



wherein x represents the number of sulfur atoms; and z and y represent the number of groups, such as from about 1 to about 6.

The thickness of the photoconductor substrate layer depends on various factors, including economical considerations, desired electrical characteristics, adequate flexibility, and the like, thus this layer may be of substantial thickness, for example over 3,000 microns, such as from about 1,000 to about 2,000 microns, from about 500 to about 1,000 microns, or from about 300 to about 700 microns, ("about" throughout includes all values in between the values recited) or of a minimum thickness. In embodiments, the thickness of this layer is from about 75 microns to about 300 microns, or from about 100 to about 150 microns. In embodiments, the photoconductor can be free of a substrate, for example the layer usually in contact with the substrate can be increased in thickness. For a photoconductor drum, the substrate or supporting medium may be of a substantial thickness of, for example, up to many centimeters or of a minimum thickness

of less than a millimeter. Similarly, a flexible belt may be of a substantial thickness of, for example, about 250 micrometers, or of a minimum thickness of less than about 50 micrometers provided there are no adverse effects on the final electrophotographic device.

Also, the photoconductor may, in embodiments, include a blocking layer, an adhesive layer, a top overcoating protective layer, and an anticurl backing layer.

The photoconductor substrate may be opaque, substantially opaque, or substantially transparent, and may comprise any suitable material that, for example, permits the photoconductor layers to be supported. Accordingly, the substrate may comprise a number of known layers, and more specifically, the substrate can be comprised of an electrically nonconductive or conductive material such as an inorganic or an organic composition. As electrically nonconducting materials, there may be selected various resins known for this purpose including polyesters, polycarbonates, polyamides, polyurethanes, and the like, which are flexible as thin webs. An electrically 10 conducting substrate may comprise any suitable metal of, for example, aluminum, nickel, steel, copper, and the like, or a polymeric material, filled with an electrically conducting substance, such as carbon, metallic powder, and the like, or an organic electrically conducting material. The electrically 15 insulating or conductive substrate may be in the form of an endless flexible belt, a web, a rigid cylinder, a sheet, and the like.

In embodiments where the substrate layer is to be rendered conductive, the surface thereof may be rendered electrically 20 conductive by an electrically conductive coating. The conductive coating may vary in thickness depending upon the optical transparency, degree of flexibility desired, and economic factors, and in embodiments this layer can be of a thickness of from about 0.05 micron to about 5 microns.

Illustrative examples of substrates are as illustrated herein, and more specifically, supporting substrate layers selected for the photoconductors of the present disclosure comprise a layer of insulating material including inorganic or organic polymeric materials, such as MYLAR® a commercially 25 available polymer, MYLAR® containing titanium, a layer of an organic or inorganic material having a semiconductive surface layer, such as indium tin oxide, or aluminum arranged thereon, or a conductive material inclusive of aluminum, chromium, nickel, brass, or the like. The substrate may be 30 flexible, seamless, or rigid, and may have a number of many different configurations, such as for example, a plate, a cylindrical drum, a scroll, an endless flexible belt, and the like. In embodiments, the substrate is in the form of a seamless flexible belt. In some situations, it may be desirable to coat on the back of the substrate, particularly when the substrate is a 35 flexible organic polymeric material, an anticurl layer, such as for example polycarbonate materials commercially available as MAKROLON®.

Generally, the photogenerating layer can contain known 40 photogenerating pigments, such as metal phthalocyanines, metal free phthalocyanines, and more specifically, alkylhydroxyl gallium phthalocyanines, hydroxygallium phthalocyanines, chlorogallium phthalocyanines, perylenes, especially bis(benzimidazo)perylene, titanyl phthalocyanines, and the like, and yet more specifically, vanadyl phthalocyanines, Type V hydroxygallium phthalocyanines, and inorganic components such as selenium, selenium alloys, and trigonal selenium. The photogenerating pigment can be dispersed in a resin binder similar to the resin binders selected 45 for the charge transport layer, or alternatively no resin binder need be present. Generally, the thickness of the photogenerating layer depends on a number of factors, including the

thicknesses of the other layers and the amount of photogenerating material contained in the photogenerating layer. Accordingly, this layer can be of a thickness of, for example, from about 0.05 micron to about 10 microns, and more specifically, from about 0.25 micron to about 2 microns when, for example, the photogenerating compositions are present in an amount of from about 30 to about 75 percent by volume.

The photogenerating composition or pigment is present in the resinous binder composition in various amounts, inclusive of 100 percent by weight based on the weight of the photogenerating components that are present. Generally, however, from about 5 percent by volume to about 95 percent by volume of the photogenerating pigment is dispersed in about 95 percent by volume to about 5 percent by volume of the resinous binder, or from about 20 percent by volume to about 30 percent by volume of the photogenerating pigment is dispersed in about 70 percent by volume to about 80 percent by volume of the resinous binder composition. In one embodiment, about 90 percent by volume of the photogenerating pigment is dispersed in about 10 percent by volume of the resinous binder composition, and which resin may be selected from a number of known polymers, such as poly(vinyl butyral), poly(vinyl carbazole), polyesters, polycarbonates, poly(vinyl chloride), polyacrylates and methacrylates, copolymers of vinyl chloride and vinyl acetate, phenolic resins, polyurethanes, poly(vinyl alcohol), polyacrylonitrile, polystyrene, and the like. It is desirable to select a coating solvent that does not substantially disturb or adversely affect the other previously coated layers of the device. Examples of coating solvents for the photogenerating layer are ketones, alcohols, aromatic hydrocarbons, halogenated aliphatic hydrocarbons, ethers, amines, amides, esters, and the like. Specific solvent examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, tetrahydrofuran, dioxane, diethyl ether, dimethyl formamide, dimethyl acetamide, butyl acetate, ethyl acetate, methoxyethyl acetate, and the like.

The photogenerating layer may comprise amorphous films of selenium and alloys of selenium and arsenic, tellurium, germanium, and the like; hydrogenated amorphous silicon, and compounds of silicon and germanium, carbon, oxygen, nitrogen, and the like fabricated by vacuum evaporation or deposition. The photogenerating layer may also comprise inorganic pigments of crystalline selenium and its alloys; Groups II to VI compounds; and organic pigments such as quinacridones, polycyclic pigments such as dibromoanthrone pigments, perylene and perinone diamines, polynuclear aromatic quinones, azo pigments including bis-, tris- and tetrakis-azos, and the like dispersed in a film forming polymeric binder and fabricated by solvent coating techniques.

In embodiments, examples of polymeric binder materials that can be selected as the matrix for the photogenerating layer components are known and include thermoplastic and thermosetting resins, such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, poly(phenylene sulfides), poly(vinyl acetate), polysiloxanes, polyacrylates, polyvinyl acetals, polyamides, polyimides, amino resins, phenoxy resins, epoxy resins, phenolic resins, polystyrene, and acrylonitrile copolymers, poly(vinyl chloride), vinyl chloride and vinyl acetate copolymers, acrylate copolymers, alkyd resins, cellulosic film formers, poly-

(amideimide), styrenebutadiene copolymers, vinylidene chloride-vinyl chloride copolymers, vinyl acetate-vinylidene chloride copolymers, styrene-alkyd resins, poly(vinyl carbazole), and the like. These polymers may be block, random, or alternating copolymers.

Various suitable and conventional known processes may be used to mix, and thereafter apply the photogenerating layer coating mixture, like spraying, dip coating, roll coating, wire wound rod coating, vacuum sublimation, and the like. For some applications, the photogenerating layer may be fabricated in a dot or line pattern. Removal of the solvent of a solvent-coated layer may be effected by any known conventional techniques such as oven drying, infrared radiation drying, air drying, and the like.

The dopant in embodiments can be added to the photogenerating dispersion, and such dopant is, more specifically, substantially dissolved in the photogenerating layer dispersion solvent.

The final dry thickness of the photogenerating layer is as illustrated herein, and can be, for example, from about 0.01 to about 30 microns after being dried at, for example, about 40° C. to about 150° C. for about 15 to about 90 minutes. More specifically, a photogenerating layer of a thickness, for example, of from about 0.1 to about 30, or from about 0.5 to about 2 microns can be applied to or deposited on the substrate, on other surfaces in between the substrate and the charge transport layer, and the like. A charge blocking layer or hole blocking layer may optionally be applied to the electrically conductive surface prior to the application of a photogenerating layer. When desired, an adhesive layer may be included between the charge blocking or hole blocking layer or interfacial layer, and the photogenerating layer. Usually, the photogenerating layer is applied onto the blocking layer and a charge transport layer, or plurality of charge transport layers are formed on the photogenerating layer. This structure may have the photogenerating layer on top of or below the charge transport layer.

In embodiments, a suitable known adhesive layer can be included in the photoconductor. Typical adhesive layer materials include, for example, polyesters, polyurethanes, and the like. The adhesive layer thickness can vary, and in embodiments is, for example, from about 0.05 micrometer (500 Angstroms) to about 0.3 micrometer (3,000 Angstroms). The adhesive layer can be deposited on the hole blocking layer by spraying, dip coating, roll coating, wire wound rod coating, gravure coating, Bird applicator coating, and the like. Drying of the deposited coating may be effected by, for example, oven drying, infrared radiation drying, air drying, and the like.

As the adhesive layers usually in contact with or situated between the hole blocking layer and the photogenerating layer, there can be selected various known substances inclusive of copolyesters, polyamides, poly(vinyl butyral), poly(vinyl alcohol), polyurethane, and polyacrylonitrile. This layer is, for example, of a thickness of from about 0.001 micron to about 1 micron, or from about 0.1 to about 0.5 micron. Optionally, this layer may contain effective suitable amounts, for example from about 1 to about 10 weight percent, of conductive and nonconductive particles, such as zinc oxide, titanium dioxide, silicon nitride, carbon black, and the like, to provide, for example, in embodiments of the present disclosure further desirable electrical and optical properties.

The hole blocking or undercoat layer for the imaging members of the present disclosure can contain a number of components including known hole blocking components, such as amino silanes, doped metal oxides, a metal oxide like titanium, chromium, zinc, tin and the like; a mixture of phenolic

compounds and a phenolic resin or a mixture of two phenolic resins, and optionally a dopant such as  $\text{SiO}_2$ . The phenolic compounds usually contain at least two phenol groups, such as bisphenol A (4,4'-isopropylidenediphenol), E (4,4'-ethylenediphenol), F (bis(4-hydroxyphenyl)methane), M (4,4'-(1,3-phenylenediisopropylidene)bisphenol), P (4,4'-(1,4-phenylene diisopropylidene)bisphenol), S (4,4'-sulfonyldiphenol), and Z (4,4'-cyclohexylidenebisphenol); hexafluorobisphenol A (4,4'-(hexafluoro isopropylidene) diphenol), resorcinol, hydroxyquinone, catechin, and the like.

The hole blocking layer can be, for example, comprised of from about 20 weight percent to about 80 weight percent, and more specifically, from about 55 weight percent to about 65 weight percent of a suitable component like a metal oxide, such as  $\text{TiO}_2$ , from about 20 weight percent to about 70 weight percent, and more specifically, from about 25 weight percent to about 50 weight percent of a phenolic resin; from about 2 weight percent to about 20 weight percent and, more specifically, from about 5 weight percent to about 15 weight percent of a phenolic compound preferably containing at least two phenolic groups, such as bisphenol S, and from about 2 weight percent to about 15 weight percent, and more specifically, from about 4 weight percent to about 10 weight percent of a plywood suppression dopant, such as  $\text{SiO}_2$ . The hole blocking layer coating dispersion can, for example, be prepared as follows. The metal oxide/phenolic resin dispersion is first prepared by ball milling or dynamilling until the median particle size of the metal oxide in the dispersion is less than about 10 nanometers, for example from about 5 to about 9. To the above dispersion are added a phenolic compound and dopant followed by mixing. The hole blocking layer coating dispersion can be applied by dip coating or web coating, and the layer can be thermally cured after coating. The hole blocking layer resulting is, for example, of a thickness of from about 0.01 micron to about 30 microns, and more specifically, from about 0.1 micron to about 8 microns. Examples of phenolic resins include formaldehyde polymers with phenol, p-tert-butylphenol, cresol, such as VARCUM™ 29159 and 29101 (available from OxyChem Company), and DURITE™ 97 (available from Borden Chemical); formaldehyde polymers with ammonia, cresol and phenol, such as VARCUM™ 29112 (available from OxyChem Company); formaldehyde polymers with 4,4'-(1-methylethylidene)bisphenol, such as VARCUM™ 29108 and 29116 (available from OxyChem Company); formaldehyde polymers with cresol and phenol, such as VARCUM™ 29457 (available from OxyChem Company), DURITE™ SD-423A, SD-422A (available from Borden Chemical); or formaldehyde polymers with phenol and p-tert-butylphenol, such as DURITE™ ESD 556C (available from Borden Chemical).

The hole blocking layer may be applied to the substrate. Any suitable and conventional blocking layer capable of forming an electronic barrier to holes between the adjacent photoconductive layer (or electrophotographic imaging layer), and the underlying conductive surface of substrate may be selected.

A number of charge transport compounds can be included in the charge transport layer, which layer generally is of a thickness of from about 5 microns to about 75 microns, and more specifically, of a thickness of from about 10 microns to about 40 microns. Examples of charge transport components are aryl amines of the following formulas/structures



wherein X is a suitable hydrocarbon like alkyl, alkoxy, aryl, and derivatives thereof; a halogen, or mixtures thereof, and especially those substituents selected from the group consisting of Cl and  $\text{CH}_3$ ; and molecules of the following formulas



wherein X, Y and Z are independently alkyl, alkoxy, aryl, a halogen, or mixtures thereof, and wherein at least one of Y and Z are present.

Alkyl and alkoxy contain, for example, from 1 to about 25 carbon atoms, and more specifically, from 1 to about 12 carbon atoms, such as methyl, ethyl, propyl, butyl, pentyl, and the corresponding alkoxides. Aryl can contain from 6 to about 36 carbon atoms, such as phenyl, and the like. Halogen includes chloride, bromide, iodide, and fluoride. Substituted alkyls, alkoxy, and aryls can also be selected in embodiments.

Examples of specific aryl amines that can be selected for the charge transport layer include  $\text{N,N}'\text{-diphenyl-N,N}'\text{-bis(alkylphenyl)-1,1-biphenyl-4,4'-diamine}$  wherein alkyl is selected from the group consisting of methyl, ethyl, propyl, butyl, hexyl, and the like;  $\text{N,N}'\text{-diphenyl-N,N}'\text{-bis(halophenyl)-1,1-biphenyl-4,4'-diamine}$  wherein the halo substituent is a chloro substituent;  $\text{N,N}'\text{-bis(4-butylphenyl)-N,N}'\text{-di-p-tolyl-[p-terphenyl]-4,4''-diamine}$ ,  $\text{N,N}'\text{-bis(4-butylphenyl)-N,N}'\text{-di-m-tolyl-[p-terphenyl]-4,4''-diamine}$ ,  $\text{N,N}'\text{-bis(4-butylphenyl)-N,N}'\text{-di-o-tolyl-[p-terphenyl]-4,4''-diamine}$ ,  $\text{N,N}'\text{-bis(4-butylphenyl)-N,N}'\text{-bis-(4-isopropylphenyl)-[p-terphenyl]-4,4''-diamine}$ ,  $\text{N,N}'\text{-bis(4-butylphenyl)-N,N}'\text{-bis(2-ethyl-6-methylphenyl)-[p-terphenyl]-4,4''-diamine}$ ,  $\text{N,N}'\text{-bis(4-butylphenyl)-N,N}'\text{-bis-(2,5-dimethylphenyl)-[p-terphenyl]-4,4''-diamine}$ ,  $\text{N,N}'\text{-diphenyl-N,N}'\text{-bis(3-$

## 11

chlorophenyl)-[p-terphenyl]-4,4"-diamine, and the like. Other known charge transport layer molecules can be selected, reference for example, U.S. Pat. Nos. 4,921,773 and 4,464,450, the disclosures of which are totally incorporated herein by reference.

Specific examples of polymer binder materials include polycarbonates, polyarylates, acrylate polymers, vinyl polymers, cellulose polymers, polyesters, polysiloxanes, polyamides, polyurethanes, poly(cyclo olefins), epoxies, and random, or alternating copolymers thereof; and more specifically, polycarbonates such as poly(4,4'-isopropylidene-diphenylene)carbonate (also referred to as bisphenol-A-polycarbonate), poly(4,4'-cyclohexylidinediphenylene) carbonate (also referred to as bisphenol-Z-polycarbonate), poly(4,4'-isopropylidene-3,3'-dimethyl-diphenyl) carbonate (also referred to as bisphenol-C-polycarbonate), and the like. In embodiments, electrically inactive binders are comprised of polycarbonate resins with a molecular weight of from about 20,000 to about 100,000, or with a molecular weight  $M_w$  of from about 50,000 to about 100,000. Generally, the transport layer contains from about 10 to about 75 percent by weight of the charge transport material, and more specifically, from about 35 percent to about 50 percent of this material.

The charge transport layer or layers, and more specifically, a first charge transport in contact with the photogenerating layer, and thereover a top or second charge transport overcoating layer may comprise charge transporting small molecules dissolved or molecularly dispersed in a film forming electrically inert polymer such as a polycarbonate. In embodiments, "dissolved" refers, for example, to forming a solution in which the small molecule is dissolved in the polymer to form a homogeneous phase; and "molecularly dispersed in embodiments" refers, for example, to charge transporting molecules dispersed in the polymer, the small molecules being dispersed in the polymer on a molecular scale. Various charge transporting or electrically active small molecules may be selected for the charge transport layer or layers. In embodiments, charge transport refers, for example, to charge transporting molecules as a monomer that allows the free charge generated in the photogenerating layer to be transported across the transport layer.

Examples of hole transporting molecules present, for example, in an amount of from about 50 to about 75 weight percent, include, for example, pyrazolines such as 1-phenyl-3-(4'-diethylamino styryl)-5-(4"-diethylamino phenyl)pyrazoline; aryl amines such as N,N'-diphenyl-N,N'-bis(3-methylphenyl)-(1,1'-biphenyl)-4,4"-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis(4-isopropylphenyl)-[p-terphenyl]-4,4"-diamine, N,N'-bis(4-butylphenyl)-N,N'-bis(2-ethyl-6-methylphenyl)-[p-terphenyl]-4,4"-diamine, N,N'-bis(4-butylphenyl)-N,N'-bis(2,5-dimethylphenyl)-[p-terphenyl]-4,4"-diamine, and N,N'-bis(2,5-dimethylphenyl)-[p-terphenyl]-4,4"-diamine, or mixtures thereof. If desired, the charge transport material in the charge transport layer may comprise a polymeric charge transport material or a combination of a small molecule charge transport material and a polymeric charge transport material.

layer with short transit times includes N,N'-diphenyl-N,N'-bis(3-methylphenyl)-(1,1'-biphenyl)-4,4"-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis(4-isopropylphenyl)-[p-terphenyl]-4,4"-diamine, N,N'-bis(4-butylphenyl)-N,N'-bis(2-ethyl-6-methylphenyl)-[p-terphenyl]-4,4"-diamine, N,N'-bis(4-butylphenyl)-N,N'-bis(3-chlorophenyl)-[p-terphenyl]-4,4"-diamine, or mixtures thereof. If desired, the charge transport material in the charge transport layer may comprise a polymeric charge transport material or a combination of a small molecule charge transport material and a polymeric charge transport material.

Examples of components or materials optionally incorporated into the charge transport layers, or at least one charge transport layer to, for example, enable improved lateral charge migration (LCM) resistance include hindered phenolic antioxidants, such as tetrakis methylene(3,5-di-tert-butyl-4-hydroxy hydrocinnamate) methane (IRGANOX<sup>TM</sup> 1010, available from Ciba Specialty Chemical), butylated hydroxytoluene (BHT), and other hindered phenolic antioxidants including SUMILIZER<sup>TM</sup> BHT-R, MDP-S, BBM-S, WX-R, NW, BP-76, BP-101, GA-80, GM and GS (available from Sumitomo Chemical Co., Ltd.), IRGANOX<sup>TM</sup> 1035, 1076, 1098, 1135, 1141, 1222, 1330, 1425WL, 1520L, 245, 259, 3114, 3790, 5057 and 565 (available from Ciba Specialties Chemicals), and ADEKA STAB<sup>TM</sup> AO-20, AO-30, AO-40, AO-50, AO-60, AO-70, AO-80 and AO-330 (available from Asahi Denka Co., Ltd.); hindered amine antioxidants such as SANOL<sup>TM</sup> LS-2626, LS-765, LS-770 and LS-744 (available from SNKYO CO., Ltd.), TINUVIN<sup>TM</sup> 144 and 622LD (available from Ciba Specialties Chemicals), MARK<sup>TM</sup> LA57, LA67, LA62, LA68 and LA63 (available from Asahi Denka Co., Ltd.), and SUMILIZER<sup>TM</sup> PS (available from Sumitomo Chemical Co., Ltd.); thioether antioxidants such as SUMILIZER<sup>TM</sup> TP-D (available from Sumitomo Chemical Co., Ltd.); phosphite antioxidants such as MARK<sup>TM</sup> 2112, PEP-8, PEP-24G, PEP-36, 329K and HP-10 (available from Asahi Denka Co., Ltd.); other molecules such as bis(4-diethylamino-2-methylphenyl)phenylmethane (BDETPM), bis-[2-methyl-4-(N-2-hydroxyethyl-N-ethylaminophenyl)]-phenylmethane (DHTPM), and the like. The weight percent of the antioxidant in at least one of the charge transport layers is from about 0 to about 20, from about 1 to about 10, or from about 3 to about 8 weight percent.

A number of processes may be used to mix, and thereafter apply the charge transport layer or layers coating mixture to the photogenerating layer. Typical application techniques include spraying, dip coating, roll coating, wire wound rod coating, and the like. Drying of the charge transport deposited coating may be effected by any suitable conventional technique such as oven drying, infrared radiation drying, air drying, and the like.

The thickness of each of the charge transport layers in embodiments is from about 10 to about 70 micrometers, but thicknesses outside this range may in embodiments also be selected. The charge transport layer should be an insulator to the extent that an electrostatic charge placed on the hole transport layer is not conducted in the absence of illumination at a rate sufficient to prevent formation and retention of an electrostatic latent image thereon. In general, the ratio of the thickness of the charge transport layer to the photogenerating layer can be from about 2:1 to 200:1, and in some instances 400:1. The charge transport layer is substantially nonabsorb-

ing to visible light or radiation in the region of intended use, but is electrically "active" in that it allows the injection of photogenerated holes from the photoconductive layer, or photogenerating layer, and allows these holes to be transported through itself to selectively discharge a surface charge on the surface of the active layer. Typical application techniques include spraying, dip coating, roll coating, wire wound rod coating, and the like. Drying of the deposited coating may be effected by any suitable conventional technique, such as oven drying, infrared radiation drying, air drying, and the like. An optional overcoating may be applied over the charge transport layer to provide abrasion protection.

Aspects of the present disclosure relate to a photoconductive imaging member comprised of a supporting substrate, an additive containing photogenerating layer, a charge blocking containing charge transport layer, and an overcoating charge transport layer; a photoconductive member with a photogenerating layer of a thickness of from about 0.1 to about 10 microns, and at least one transport layer each of a thickness of from about 5 to about 100 microns; a member wherein the thickness of the photogenerating layer is from about 0.1 to about 4 microns; a member wherein the photogenerating layer contains a polymer binder; a member wherein the binder is present in an amount of from about 50 to about 90 percent by weight, and wherein the total of all layer components is about 100 percent; a member wherein the photogenerating component is a hydroxygallium phthalocyanine that absorbs light of a wavelength of from about 370 to about 950 nanometers; an imaging member wherein the supporting substrate is comprised of a conductive substrate comprised of a metal; an imaging member wherein the conductive substrate is aluminum, aluminized polyethylene terephthalate, or titanized polyethylene terephthalate; a photoconductor wherein the photogenerating resinous binder is selected from the group consisting of polyesters, polyvinyl butyral, polycarbonates, polystyrene-*b*-polyvinyl pyridine, and polyvinyl formals; an imaging member wherein the photogenerating pigment is a metal free phthalocyanine; a photoconductor wherein the charge transport layers comprises



wherein X is selected from the group consisting of lower, that is with, for example, from 1 to about 8 carbon atoms, alkyl, alkoxy, aryl, and halogen; a photoconductor wherein each of, or at least one of the charge transport layers comprises



wherein X and Y are independently lower alkyl, lower alkoxy, phenyl, a halogen, or mixtures thereof, and wherein the photogenerating and charge transport layer resinous binder is

selected from the group consisting of polycarbonates and polystyrene; a photoconductor wherein the photogenerating pigment present in the photogenerating layer is comprised of chlorogallium phthalocyanine, or Type V hydroxygallium phthalocyanine prepared by hydrolyzing a gallium phthalocyanine precursor by dissolving the hydroxygallium phthalocyanine in a strong acid, and then reprecipitating the resulting dissolved precursor in a basic aqueous media; removing any ionic species formed by washing with water; concentrating the resulting aqueous slurry comprised of water and hydroxygallium phthalocyanine to a wet cake; removing water from the wet cake by drying; and subjecting the resulting dry pigment to mixing with the addition of a second solvent to cause the formation of the hydroxygallium phthalocyanine; an imaging member wherein the Type V hydroxygallium phthalocyanine has major peaks, as measured with an X-ray diffractometer, at Bragg angles (2 theta+/-0.2°) 7.4, 9.8, 12.4, 16.2, 17.6, 18.4, 21.9, 23.9, 25.0, 28.1 degrees, and the highest peak at 7.4 degrees; a method of imaging which comprises generating an electrostatic latent image on the photoconductor developing the latent image, and transferring the developed electrostatic image to a suitable substrate; a method of imaging wherein the imaging member is exposed to light of a wavelength of from about 370 to about 950 nanometers; a member wherein the photogenerating layer is of a thickness of from about 0.1 to about 50 microns; a member wherein the photogenerating pigment is dispersed in from about 1 weight percent to about 80 weight percent of a polymer binder; a member wherein the binder is present in an amount of from about 50 to about 90 percent by weight, and wherein the total of the layer components is about 100 percent; a photoconductor wherein the photogenerating component is Type V hydroxygallium phthalocyanine, or chlorogallium phthalocyanine, and the charge transport layer contains a hole transport of N,N'-diphenyl-N,N-bis(3-methylphenyl)-1,1'-biphenyl-4,4'-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis-(4-isopropylphenyl)-[p-terphenyl]-4,4"-diamine, N,N'-bis(4-butylphenyl)-N,N'-bis-(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, N,N'-diphenyl-N,N'-bis(3-chlorophenyl)-[p-terphenyl]-4,4"-diamine molecules, and wherein the hole transport resinous binder is selected from the group consisting of polycarbonates and polystyrene; an imaging member wherein the photogenerating layer contains a metal free phthalocyanine; a photoconductive imaging member comprised of a supporting substrate, a doped photogenerating layer, a hole transport layer, and in embodiments wherein a plurality of charge transport layers are selected, such as for example, from two to about ten, and more specifically two, may be selected; and a photoconductive imaging member comprised of an optional supporting substrate, a photogenerating layer, and a first, second, and third charge transport layer.

60 The following Examples are being submitted to illustrate embodiments of the present disclosure.

#### Comparative Example 1

There was prepared a photoconductor with a biaxially oriented polyethylene naphthalate substrate (KALEDEX™ 2000) having a thickness of 3.5 mils, and thereover, a 0.02 micron thick titanium layer was coated on the biaxially oriented polyethylene naphthalate substrate (KALEDEX™

## 15

2000). Subsequently, there was applied thereon, with a gravure applicator or an extrusion coater, a hole blocking layer solution containing 50 grams of 3-aminopropyl triethoxysilane ( $\gamma$ -APS), 41.2 grams of water, 15 grams of acetic acid, 684.8 grams of denatured alcohol, and 200 grams of heptane. This layer was then dried for about 1 minute at 120° C. in a forced air dryer. The resulting hole blocking layer had a dry thickness of 500 Angstroms. An adhesive layer was then deposited by applying a wet coating over the blocking layer, using a gravure applicator or an extrusion coater, and which adhesive contained 0.2 percent by weight based on the total weight of the solution of the copolyester adhesive (ARDEL D100<sup>TM</sup> available from Toyota Hsutsu Inc.) in a 60:30:10 volume ratio mixture of tetrahydrofuran/monochlorobenzene/methylene chloride. The adhesive layer was then dried for about 1 minute at 120° C. in the forced air dryer of the coater. The resulting adhesive layer had a dry thickness of 200 Angstroms.

25 A photogenerating layer dispersion was prepared by introducing 0.45 gram of the known polycarbonate IUPILON 200<sup>TM</sup> (PCZ-200) weight average molecular weight of 20,000, available from Mitsubishi Gas Chemical Corporation, and 50 milliliters of tetrahydrofuran into a 4 ounce glass bottle. To this solution were added 2.4 grams of hydroxygallium phthalocyanine (Type V) and 300 grams of  $\frac{1}{8}$  inch (3.2 millimeters) diameter stainless steel shot. This mixture was then placed on a ball mill for 8 hours. Subsequently, 2.25 grams of PCZ-200 were dissolved in 46.1 grams of tetrahydrofuran, and added to the hydroxygallium phthalocyanine dispersion. This slurry was then placed on a shaker for 10 minutes. The resulting dispersion was, thereafter, applied to the above adhesive interface with a Bird applicator to form a photogenerating layer having a wet thickness of 0.25 mil. A strip about 10 millimeters wide along one edge of the substrate web bearing the blocking layer and the adhesive layer was deliberately left uncoated by any of the photogenerating layer material to facilitate adequate electrical contact by the ground strip layer that was applied later. The photogenerating layer was dried at 120° C. for 1 minute in a forced air oven to form a dry photogenerating layer having a thickness of about 0.3 to 0.5 micron.

30 The resulting photoconductor web was then coated with a charge transport layer prepared by introducing into an amber glass bottle in a weight ratio of 50/50, N,N'-bis(methylphenyl)-1,1-biphenyl-4,4'-diamine (TBD) and poly(4,4'-isopropylidene diphenyl)carbonate, a known bisphenol A polycarbonate having a  $M_w$  molecular weight average of about 120,000, commercially available from Farbenfabriken Bayer A.G. as MAKROLON<sup>®</sup> 5705. The resulting mixture was then dissolved in methylene chloride to form a solution containing 15.6 percent by weight solids. This solution was applied on the photogenerating layer to form the charge transport layer coating that upon drying (120° C. for 1 minute) had a thickness of 27 microns. During this coating process, the humidity was equal to or less than 30 percent, for example 25 percent.

## Example I

35 A photoconductor was prepared by repeating the process of Comparative Example 1 except that there was included in the photogenerating layer 2 weight percent of dipentamethylenethiuram tetrasulfide (DPTT) which DPTT was added to and mixed with the prepared photogenerating dispersion prior to the coating thereof on the supporting substrate. More specifically, the dipentamethylenethiuram tetrasulfide (DPTT) additive was first dissolved in the photogenerating

## 16

5 layer solvent of tetrahydrofuran, and then the resulting mixture was added to the hydroxygallium phthalocyanine Type V mixture. Thereafter, the mixture resulting was deposited on the supporting substrate.

## Example II

10 A photoconductor was prepared by repeating the process of Example I except that there was included in the photogenerating layer 5 weight percent of dipentamethylenethiuram tetrasulfide (DPTT)

## Example III

15 A photoconductor was prepared by repeating the process of Example I except that there was included in the photogenerating layer 10 weight percent of dipentamethylenethiuram tetrasulfide (DPTT).

## Example IV

20 A photoconductor was prepared by repeating the process of Example I except that there was included in the photogenerating layer 2 weight percent of N,N'-diphenylguanidine (DPG).

## Example V

25 A photoconductor was prepared by repeating the process of Example I except that there was included in the photogenerating layer 2 weight percent of zinc diethyldithiocarbamate (ZDEC).

## Example VI

30 A photoconductor was prepared by repeating the process of Example I except that there was included in the photogenerating layer 2 weight percent of TROYSOL S366, an aliphatic acid available from Troy Chemicals.

## Example VII

35 A photoconductor was prepared by repeating the process of Example I except that there was included in the photogenerating layer 2 weight percent of TROYSOL S367, an aliphatic acid available from Troy Chemicals.

## Electrical Property Testing

50 The above prepared photoconductors of Comparative Example 1 and a number of the disclosed photoconductors containing the additive were tested in a scanner set to obtain photoinduced discharge cycles, sequenced at one charge-erase cycle followed by one charge-expose-erase cycle, 55 wherein the light intensity was incrementally increased with cycling to produce a series of photoinduced discharge characteristic curves from which the photosensitivity and surface potentials at various exposure intensities were measured. Additional electrical characteristics were obtained by a series of charge-erase cycles with incrementing surface potential to generate several voltage versus charge density curves. The scanner was equipped with a scorotron set to a constant voltage charging at various surface potentials. The photoconductors were tested at surface potentials of 400 volts with the 60 exposure light intensity incrementally increased by means of regulating a series of neutral density filters; and the exposure light source was a 780 nanometer light emitting diode. The 65

xerographic simulation was completed in an environmentally controlled light tight chamber at ambient conditions (40 percent relative humidity and 22° C.).

The results are summarized in Table 1 wherein V(2.1) is the surface potential of the photoconductors at an exposure energy of 2.1 ergs/cm<sup>2</sup>; and V<sub>erase</sub> is the surface potential of the photoconductors after they were subjected to an erase light of 680 nanometers at an intensity of about 100 to about 150 ergs/cm<sup>2</sup>;  $\Delta V_{ddp}$  (5 k) is the change in dark depleted surface potential, for example, about 26 ms after charging in the dark, after subjecting the photoconductors to 5,000 cycles of repeated charging and erase cycles; and  $\Delta V2.1$  (5 k) is the change in V(2.1) after subjecting the photoconductors to 5,000 cycles of repeated charging and erase cycles. The electrical scanning results indicate that the V(2.1) and V<sub>erase</sub> of DPTT, ZDEC, TROYSOL 366 and TROYSOL 367 are similar to the Comparative Example 1, suggesting that these materials possessed no detrimental effects to the photoconductors. The DPTT also shows similar  $\Delta V_{ddp}$  (5 k) and smaller  $\Delta V2.1$  (5 k) than the Comparative Example 1, indicating that this additive can improve cyclic stability and extend the photoconductor life.

TABLE 1

| Summary of Photoelectrical and Ghosting Performances |         |                 |                       |                    |           |
|------------------------------------------------------|---------|-----------------|-----------------------|--------------------|-----------|
| Device                                               | V (2.1) | V <sub>er</sub> | $\Delta V_{ddp}$ (5k) | $\Delta V2.1$ (5k) | Ghost SIR |
| Example I<br>(2% DPTT)                               | 75      | 46              | 2                     | 6                  | 5.4       |
| Example II<br>(5% DPTT)                              | 72      | 42              | 2                     | 10                 | N/A       |
| Example III<br>(10% DPTT)                            | 72      | 41              | 3                     | 40                 | N/A       |
| Example IV<br>2% DPG                                 | 161     | 104             | N/A                   | N/A                | 8.6       |
| Example V<br>2% ZDEC                                 | 85      | 38              | N/A                   | N/A                | 7.6       |
| Example VI<br>2% S366                                | 71      | 30              | N/A                   | N/A                | 8.8       |
| Example VII<br>2% S367                               | 63      | 25              | N/A                   | N/A                | 8.0       |
| Comparative<br>Example 1                             | 67      | 30              | 5                     | 48                 | 8.0       |
| Comparative<br>Example 1<br>(repeat)                 | 78      | 44              | N/A                   | N/A                | 8.9       |

DPG: N,N'-diphenylguanidine;

ZDEC: zinc diethyldithiocarbamate,

TROYSOL S366: undisclosed aliphatic acids,

TROYSOL 367: undisclosed aliphatic acids.

### Ghosting Measurements

When a photoconductor is selectively exposed to positive charges in a xerographic print engine, such as the Xerox Corporation iGen3®, it is observed that some of these charges enter the photoconductor and manifest themselves as a latent image in the next printing cycle. This print defect can cause a change in the lightness of the half tones, and is commonly referred to as a "ghost" that is generated in the previous printing cycle.

An example of a source of the positive charges is the stream of positive ions emitted from the transfer corotron. Since the paper sheets are situated between the transfer corotron and the photoconductor, the photoconductor is shielded from the positive ions from the paper sheets. In the areas between the paper sheets, the photoconductor is fully exposed, thus in this paper free zone the positive charges may enter the photoconductor. As a result these charges cause a print defect or ghost

in a half tone print if one switches to a larger paper format that covers the previous paper free zone.

In the ghosting test the photoconductors were electrically cycled to simulate continuous printing. At the end of every tenth cycle known, incremental positive charges were injected. In the follow-on cycles the electrical response to these injected charges were measured and then translated into a rating scale.

The electrical response to the injected charges in the print engine and in the electrical test fixture was a drop in the surface potential. This drop was calibrated to colorimetric values in the prints and they in turn were calibrated to the ranking scale of an average rating of at least two observers. On this scale, 1 refers to no observable ghost, and values of 7 refer to a very strong ghost. The functional dependence between the change in surface potential and the ghosting scale is slightly supra-linear and may in first approximation be linearly scaled. Note that these tests are done under severe stress conditions, for example actuators in the print engine and in the test fixture are set as such to bring out the worst ghost.

Using a sputterer  $\frac{3}{8}$  inch diameter, 150 Å thick, gold dots were deposited onto the transport layer of the photoconductors in the Examples. Then, they were dark rested (for example, in the absence of light) for at least two days at 22° C. and 50 percent RH to allow relaxation of the surfaces.

These electroded photoconductor devices (gold dot on charge transport layer surface) were then cycled in a test fixture that injected positive charge through the gold dots with the methodology described above. The change in surface potential was then determined for injected charges of 27 nC/cm<sup>2</sup>. This value was selected to be larger than typically expected in the Xerox Corporation iGen3® print engine to generate strong signals. Finally the changes in the surface potentials were translated into ghost rankings by the aforementioned calibration curves. This method was repeated 4 times for each photoconductor tested, and then the averages were calculated. Typical standard deviation of the mean tested on numerous devices was about 0.35. The ghosting ratings are reported in Table 1 above.

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others. Unless specifically recited in a claim, steps or components of claims should not be implied or imported from the specification or any other claims as to any particular order, number, position, size, shape, angle, color, or material.

What is claimed is:

1. A photoconductor consisting of a supporting substrate, a photogenerating layer, and at least one charge transport layer comprised of at least one charge transport compound, wherein said at least one charge transport layer is comprised of a top charge transport layer and a bottom charge transport layer, and wherein said top charge transport layer is in contact with said bottom charge transport layer and said bottom charge transport layer is in contact with said photogenerating layer, each of said bottom and said top charge transport layer containing from about 50 to about 75 weight percent of said charge transport compound, and wherein said charge transport compound comprises aryl amine molecules as represented by at least one of the following formulas/structures, wherein X is selected from the group consisting of at least one of alkyl, alkoxy, aryl, and halogen, and wherein each of said bottom and said top charge transport layer includes an

19

optional antioxidant comprised of at least one of a hindered phenolic and a hindered amine



wherein X, Y and Z are independently selected from the group consisting of at least one of alkyl, alkoxy, aryl, and halogen, and wherein said photogenerating layer contains a thiram tetrasulfide additive of the following formulas/structures present in an amount of from about 0.1 to about 10 percent by weight, and which thiram tetrasulfide additive excludes dipentamethylenethiuramtetrasulfide



wherein each R is independently selected from the group consisting of at least one of hydrogen, alkoxy, and aryl, and x represents 4.

20

2. A photoconductor in accordance with claim 1 wherein said thiram tetrasulfide additive is present in an amount of from about 1 to about 5 percent by weight.

3. A photoconductor in accordance with claim 1 wherein said thiram tetrasulfide additive is present in an amount of from about 2 to about 4 percent by weight.

4. A photoconductor in accordance with claim 1 wherein said alkyl and said alkoxy for said aryl amine molecules each contains from about 1 to about 12 carbon atoms, and said aryl 10 contains from about 6 to about 36 carbon atoms, and said photogenerating layer contains a photogenerating pigment.

5. A photoconductor in accordance with claim 1 wherein said aryl amine is N,N'-diphenyl-N,N-bis(3-methylphenyl)-1,1'-biphenyl-4,4'-diamine.

15 6. A photoconductor in accordance with claim 1 wherein said charge transport compound is selected from the group consisting of N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4"-diamine, N,N'-bis(4-butylphenyl)-

20 N,N'-di-o-tolyl-[p-terphenyl]-4,4'-diamine, N,N'-bis(4-butylphenyl)-N,N'-bis-(4-isopropylphenyl)-[p-terphenyl]-4, 4'-diamine, N,N'-bis(4-butylphenyl)-N,N'-bis-(2-ethyl-6-methylphenyl)-[p-terphenyl]-4,4'-diamine, N,N'-bis(4-butylphenyl)-N,N'-bis-(2,5-dimethylphenyl)-[p-terphenyl]-25 4,4'-diamine, N,N'-diphenyl-N,N'-bis(3-chlorophenyl)-[p-terphenyl]-4,4'-diamine, and mixtures thereof.

7. A photoconductor in accordance with claim 1 wherein said antioxidant comprised of at least one of a hindered phenolic and a hindered amine is present.

30 8. A photoconductor in accordance with claim 1 wherein said photogenerating layer is comprised of at least one photogenerating pigment and said additive.

9. A photoconductor in accordance with claim 8 wherein said photogenerating pigment is comprised of at least one of a metal phthalocyanine, and a metal free phthalocyanine.

35 10. A photoconductor in accordance with claim 8 wherein said photogenerating pigment is comprised of chlorogallium phthalocyanine.

11. A photoconductor in accordance with claim 8 wherein 40 said photogenerating pigment is comprised of hydroxygallium phthalocyanine.

12. A photoconductor in accordance with claim 8 wherein said photogenerating pigment is comprised of titanyl phthalocyanine.

\* \* \* \* \*